

April 17, 1945.

A. FRÖHLICH ET AL

2,373,821

PRODUCTION OF COLOR PHOTOGRAPHIC IMAGES

Filed Feb. 17, 1942



Fig. 1.



Fig. 2.

INVENTORS  
ALFRED FROHLICH AND  
WILHELM SCHNEIDER

BY *Henry M. Lang*

ATTORNEYS

## UNITED STATES PATENT OFFICE

2,373,821

## PRODUCTION OF COLOR PHOTOGRAPHIC IMAGES

Alfred Fröhlich and Wilhelm Schneider, Dessau, Germany, assignors to General Aniline & Film Corporation, New York, N. Y., a corporation of Delaware

Application February 17, 1942, Serial No. 431,272  
In Germany October 19, 1940

12 Claims. (Cl. 95—6)

The present invention relates to the production of color photographic images and in particular of images obtained by color forming development.

In the production of color photographic images it is known to use in the photographic emulsion layer or the developer dyestuff formers which yield dyestuff images by reaction with the oxidation products of the developing substance in the development of the latent silver image. For processes of producing color images by means of a multi-layer material it is of importance to adjust the color tones of the single partial dyestuff images so that they fulfill the theoretical requirements of the subtractive tri-color process as completely as possible. This requirement must especially be satisfied for the negative-positive process which requires the use of dyestuffs having particular spectral properties. It is of the greatest importance for this process that the blue dyestuffs transmit the rays in the blue and green regions of the spectrum in a relatively large amount. Blue dyestuffs having this property have already been proposed. There are, for instance, used condensable phenols and naphthols which contain halogens as substituents. These halogen substituted products, however, have the disadvantage that their solubility is very low compared with that of the non-substituted naphthols so that it is sometimes practically impossible as, for instance, with pentabromonaphthol to obtain a sufficiently high concentration of dyestuff formers in the developer. Moreover, it has been suggested to use phenols with nitrogenous 6-membered rings fused on as, for instance, hydroxyquinolines instead of naphthols. However, it has been found that the color tone of the dyestuffs produced with these hydroxyquinolines is hardly different from the analogous dyestuffs derived from naphthol so that it is generally immaterial for practical purposes whether  $\alpha$ -naphthols or hydroxyquinolines are employed. It is furthermore known that three rings condensed together as, for instance, 1-hydroxyanthracene yield blue-green dyestuffs having a very green color tone. These compounds, however, are not suitable, for due to their extraordinary sensitivity to air, developers containing these dyestuff formers become black when exposed to air for a short time. Hydroxyphenanthrenes would likewise form greenish color tones. These compounds, however, cannot be used because they cannot be prepared as yet on a technical scale.

The present invention is based on the observation that dyestuff formers yielding quinoneimine dyestuffs which exhibit an especially high absorption in the short wave infra-red and hence satisfy the requirements of the negative process as to the spectral properties of the dyestuffs to a large extent and are moreover suitable for the purposes of sound recording owing to the high absorption in the long wave red can be produced by using as dyestuff formers condensable aromatic hydroxy compounds containing in their molecule a 5-membered heterocyclic nucleus.

From the halogenated phenols and naphthols and the o-hydroxyphenylbenzal compounds proposed as components for the blue-green the dyestuff formers of the present invention are distinguished in that they can additionally be substituted with great ease owing to their constitution. Thus they can without difficulty be substituted by radicals which are especially favorable for photographic purposes as, for instance, non-diffusing radicals and groups rendering the components soluble in diluted alkalies. Owing to the easy introduction of several substituents it is also possible to influence the color tone in any desired manner.

The heterocyclic nucleus may be a free substituent as, for instance, the 5-membered ring in the condensation product from  $\alpha$ -hydroxynaphthoic acid and nitroaminobenzthiazole corresponding with the following formula



(1-hydroxy-2-naphthoyl-5'-nitro-2'-amino-benzthiazole) and in the product obtained by condensing  $\alpha$ -hydroxynaphthoic acid with o-aminophenol and heating the reaction product to split off water and having the following formula:



(1-hydroxynaphthalene - 2,2' - benzoxazole) and in the component obtained by heating the condensation product from  $\alpha$ -hydroxynaphthoic acid

and o-phenylenediamine to split off water and having the following formula:



(1 - hydroxynaphthalene - 2,2' - benzimidazole).

The heterocyclic nucleus may also directly be fused on the phenol or naphthol capable of coupling as, for instance, in hydroxynaphthylamino-phenylthiazole sulfonic acid of the following formula:



This compound and the homologues thereof are prepared in known manner as, for instance, according to the process described in the German Patent 165,126.

The preferred compounds according to the present invention are salts of phenols having joined thereto in ortho position to the phenolic hydroxyl group a radical such as a benzthiazole, a benzoxazole or a benzimidazole, the carbon atom between the hetero atoms of the five-membered ring of such heterocyclic radical being linked to the phenol through a nuclear carbon to carbon linkage and said salt having linked thereto a radical rendering the salt fast to diffusion in gelatin. Examples of such compounds are given above.

Reference is made to the accompanying drawing the two figures of which show absorption curves of dyestuff formed from p-dimethylaminoaniline and dyestuff components of the present invention compared to absorption curves of dyestuffs from known dyestuff formers.

For the production of non-diffusing components radicals producing fastness to diffusion may be introduced into the dyestuff formers according to U. S. Patents 2,186,852, 2,186,851, 2,186,849, 2,186,734, 2,186,733, 2,186,732 dated January 9, 1940, U. S. Patents 2,179,244, 2,186,719, 2,178,612 dated November 7, 1939, and U. S. Patents 2,280,722, 2,292,575, 2,307,399, 2,303,928, 2,357,393, 2,341,372 and 2,323,590. Italian Patents 344,649, 344,648, French Patent 844,637, and U. S. Patent applications, Serial Nos. 284,258, filed July 13, 1939, and 333,814 filed May 7, 1940.

The silver halide emulsion prepared by means of the non-diffusing dyestuff formers may be cast to form single layers or worked up into multi-layer materials containing the several emulsion layers on one or both sides of the support and, if necessary, filter layers, intermediate layers or anti-halation layers.

#### Example

Into 1-hydroxynaphthyl-5,6-3'-aminophenylthiazole-2-sulfonic acid prepared in the manner described in German Patent 165,126 a radical preventing diffusion may be introduced by reacting the dyestuff component with stearic acid chloride or abietic acid chloride or perhydrodiphenylcarboxylic acid chloride. Owing to the presence of the sulfo group the non-diffusing

dyestuff former thus obtained possesses good solubility.

For the production of color images 3 g. of the dyestuff former are dissolved in a mixture of 5 100 cc. of water and 10 cc. of n/1 sodium hydroxide solution. The obtained solution is then added to 300 cc. of a silver halide gelatin emulsion whereupon the emulsion is usually cast to form a layer. The exposed layer is treated with a color forming developer as, for instance, p-dimethylaminoaniline in soda-alkaline solution. After fixing and removing the silver one obtains a green dyestuff image.

Instead of the sodium salt other soluble salts 15 of the dyestuff former may be used, for instance, other alkali metal salts.

In Figure 1 the curve 1 represents the absorption 20 curve of the dyestuff formed from 1'-hydroxy-2'-naphthyl-2-benzimidazole-4'-sulfonic acid and p-dimethylaminoaniline and the curve 2 the absorption curve of the dyestuff formed from 1'-hydroxy-2'-naphthyl-2-benzoxazole and p-dimethylaminoaniline. The curves 3 and 4 represent the absorption curves of the dyestuffs from 25 the known dyestuff formers  $\alpha$ -naphthol and 2,4-dibromonaphthol respectively.

In Figure 2 the absorption curve 1 is that of the dyestuff from 1-hydroxynaphthyl-5,6-3'-aminophenylthiazole-2-sulfonic acid whereas the 30 curves 2 and 3 are the absorption curves of the dyestuffs from  $\alpha$ -naphthol and 2,4-dibromonaphthol respectively.

We claim:

1. In a process of producing color photographic 35 images by color forming development, the improvement which comprises developing an exposed silver halide emulsion with an aromatic primary amino developer in the presence of a water-soluble salt of a phenol having joined

40 thereto in ortho position to the phenolic hydroxyl group a radical selected from the class consisting of benzthiazole, benzoxazole and benzimidazole radicals, the carbon atom between the hetero atoms of the five-membered ring of said radical being linked to said phenol through a nuclear carbon to carbon linkage.

2. In a process of producing color photographic 45 images by color forming development, the improvement which comprises developing an exposed photographic silver halide emulsion with an aromatic primary amino developer containing a soluble salt of a phenol having joined thereto in ortho position to the phenolic hydroxyl group a radical selected from the class consisting of benzthiazole, benzoxazole and benzimidazole radicals, the carbon atom between the hetero atoms of the five-membered ring of said radical being linked to said phenol through a nuclear carbon to carbon linkage.

3. In a process of producing color photographic 50 images by color forming development, the improvement which comprises developing with an aromatic primary amino developer, a silver halide emulsion containing a soluble salt of a phenol having joined thereto in ortho position to the phenolic hydroxyl group a radical selected from the class consisting of benzthiazole, benzoxazole and benzimidazole radicals, the carbon atom between the hetero atoms of the five-membered ring of said radical being linked to said phenol through a nuclear carbon to carbon linkage.

4. A silver halide gelatin emulsion for color 55 forming development containing a soluble salt of a phenol having joined thereto in ortho position to the phenolic hydroxyl group a radical se-

lected from the class consisting of benzthiazole, benzoxazole and benzimidazole radicals, the carbon atom between the hetero atoms of the five-membered ring of said radical being linked to said phenol through a nuclear carbon to carbon linkage.

5. A color forming developer comprising an aqueous solution containing an aromatic primary amino developing agent and a soluble salt of a phenol having joined thereto in ortho position to the phenolic hydroxyl group a radical selected from the class consisting of benzthiazole, benzoxazole and benzimidazole radicals, the carbon atom between the hetero atoms of the five-membered ring of said radical being linked to said phenol through a nuclear carbon to carbon linkage.

6. In a process of producing color photographic images by color-forming development, the improvement which comprises developing an exposed silver halide emulsion with an aromatic primary amino developer in the presence of a salt of a phenol having joined thereto in ortho position to the phenolic hydroxyl group a radical selected from the class consisting of benzthiazole, benzoxazole and benzimidazole radicals, the carbon atom between the hetero atoms of the five-membered ring of said radical being linked to said phenol through a nuclear carbon to carbon linkage, said salt having joined thereto a radical rendering the salt fast to diffusion.

7. A silver halide gelatin emulsion for color-forming development containing a salt of a phenol having joined thereto in ortho position to the phenolic hydroxyl group a radical selected

from the class consisting of benzthiazole, benzoxazole and benzimidazole radicals, the carbon atom between the hetero atoms of the five-membered ring of said radical being linked to said phenol through a nuclear carbon to carbon linkage, said salt containing a radical rendering the salt fast to diffusion.

8. The process as defined in claim 1 wherein said phenol is a naphthol.

10. The process as defined in claim 2 wherein said phenol is a naphthol.

15. The composition as defined in claim 4 wherein said phenol is a naphthol.

11. A silver halide emulsion for color-forming development containing a compound of the following constitution:



20. 12. A silver halide emulsion for color forming development containing a compound of the following constitution:



25. ALFRED FRÖHLICH.  
WILHELM SCHNEIDER.